

Patented Dec. 7, 1943

2,336,014

# UNITED STATES PATENT OFFICE

2,336,014

## FROTH FLOTATION OF CEMENT RAW MATERIALS

David Walker Jayne, Jr., Old Greenwich, Stephen Edward Erickson, Springdale, and Harold Milton Day, Cos Cob, Conn., assignors to American Cyanamid Company, New York, N. Y., a corporation of Maine

No Drawing. Application September 28, 1940,  
Serial No. 358,830

11 Claims. (Cl. 209—166)

This invention relates to the froth flotation treatment of cement raw materials and more particularly to the concentration of calcite from the usual gangue minerals found in argillaceous limestones, marls, and chalks to produce concentrates useful in the manufacture of Portland cement.

It has been known in the past that calcite could be concentrated by froth flotation operations in which the flotation was carried out in the presence of fatty acid oxide mineral collecting reagents, such as oleic acid and fish oil fatty acids. While these fatty acids have been used extensively, they are not entirely satisfactory in that it is very difficult to obtain satisfactory dispersion in the ore pulps and they cannot be effectively used in cold water. Also they are unsatisfactory for the concentration of very fine particles of calcite and particularly at normal pulp temperature which is believed to be due, at least in part, to incomplete dispersion and over-oiling which causes flocculation of the gangue materials resulting in concentrates of low grade. Emulsions of the above fatty acids are also not entirely satisfactory since they have a tendency to produce excessive frothing which results in the production of low grade concentrates. Similarly the sodium soaps of oleic acid and fish oil fatty acids result in the production of excessive froths of low grade which are inefficient as calcite collectors.

In accordance with the present invention we have found that the sodium salts or soaps of fatty acids containing less than 18 carbon atoms and preferably 8 to 16 carbon atoms are efficient calcite promoters in spite of the general belief heretofore that sodium soaps could not be successfully used. The general experience in the past has been that oxide minerals such as phosphate rock could not be effectively promoted using the sodium soaps of oleic acid or those of fish oil fatty acids whereas they could be when the acids and alkali were added to the ore pulp separately. We have found, however, that the sodium soaps of individual fatty acids containing from 8 to 16 carbon atoms, examples of which are sodium laurate, sodium myristate, and sodium palmitate, and the sodium soaps of mixtures of fatty acids in which the mixtures are made up of at least one third fatty acids containing not more than 16 carbon atoms, examples of which are the sodium soaps of the fatty acids of coconut oil, palm kernel oil, and palm oil, are selective calcite promoters and are more effective than the common fatty acids such as fish oil fatty acids and oleic acid now widely used.

The reagents of the present invention are very easily dispersed in aqueous ore pulps even at low temperatures which is of decided value because it eliminates the necessity for the use of warm water in ore pulps as often required when the

ordinary fatty acids are employed as collectors. It is also an advantage of the present invention that our reagents are cheap, particularly the sodium soaps of coconut oil, palm kernel oil, and palm oil, which are produced simply by saponifying the respective oils with sodium hydroxide; and it is not necessary to remove the glycerine split off in the saponification reaction since the glycerine does not appear to materially affect the promoter action.

Among the purposes of the invention are to provide a low cost but highly selective calcite collecting reagent; to extend the practical use of flotation for the economical recovery of calcite from minerals of low commercial value, and to permit the recovery of useful concentrates from slimy pulps which do not react successfully to froth flotation with the fatty acid collectors. Some of the advantages of our reagents are that they can be diluted in water to any convenient degree to make possible light and uniform stage oiling; they are stable at all working temperatures and are quickly dispersed even in ice water; and they are highly selective. These advantages extend the practical use of flotation to the recovery of the valuable content of cement raw materials such as the extremely fine grained material described as "blue limestone" of the Lehigh Valley district of Pennsylvania which are not readily amenable to flotation to produce concentrates of commercial grades, with the usual collectors, such as oleic acid, fish oil fatty acids, resin acids, soaps or emulsions, or mixtures thereof.

The principal minerals present in cement raw materials are calcite; silica in the form of quartz, flint and/or chalcedony; silicates of alumina, usually one or more forms of mica, but frequently as talc, feldspar, etc.; iron oxides, limonite and/or pyrite, and magnesia as dolomite, brucite, and/or combined with silicates of alumina, as for example phlogopite. In addition, minor quantities of other minerals are frequently present. The objectives in processing such materials are to recover a maximum of the available calcite and silica, and usually iron, and to eliminate all but a minor quantity of the compounds of alumina, including the magnesian silicates of alumina, whereby the recovered constituents may be utilized as a cement raw material mixture, or the major part thereof, for the production of modern cements, particularly those of low heat of hydration and resistant to sulphates. It may be said, therefore, that Portland cement raw materials comprise essentially a mixture of silica, alumina, iron, and calcium carbonate and to be commercially useful the calcium carbonate should represent about 77% of the total. In the beneficiation of cement raw material it is desirable to obtain high weight recovery of the calcite of at least about 76% purity.

and at the same time reject a high proportion of the argillaceous compounds, usually silicates of alumina and quartz. It has been difficult in the past to economically produce concentrates conforming to the above standards using the ordinary fatty acid type calcite collectors. The following examples are specific illustrations of the present invention in which satisfactory concentrates were produced under economical conditions. It is to be understood, however, that the invention is not to be limited by the specific conditions set forth in the examples.

Comparative froth flotation tests were conducted with various reagent combinations on a sample of cement raw material of the Lehigh Valley Bluestone type in the following manner.

The ore charge was ground to 93% minus 325 mesh and 1.76% plus 200 mesh in a rod mill. The ground pulp was placed in a Fagergren flotation machine, diluted to 22% solids and conditioned for one minute with 1.0 lb. of calcium lignin sulfonate per ton of ore. A concentrate was then floated by the addition (in 7 stages) of small amounts of the promoter being tested. The total time of flotation was 7 minutes. The results obtained are given in the following table.

The results in the above table indicate that only 0.5 pound of the sodium soap of coconut oil fatty acid per ton of ore produced results which are better than those produced by using 2.00 pounds per ton of ore of fish oil fatty acids or talloel.

The improved calcite promoter of the present invention may be used in conjunction with recent developments in the treatment of cement raw materials. For example, when carbonaceous materials are to be treated the carbon may be first dispersed by the addition of carbon dispersers, such as calcium lignin sulfonate prior to the froth flotation using the promoter of the present invention. The promoters may likewise be used in processes in which the froth flotation tails are subsequently subjected to a froth flotation treatment in the presence of a cationic promoter to reduce the silica content.

In the above flotation tests it is seen that the low molecular weight sodium soap of coconut oil is a much better calcite collector than the high molecular weight soap of cottonseed oil. In similar tests we have determined that the sodium soaps of palm oil and palm kernel oil are efficient calcite promoters, whereas the sodium soaps of oils such as cottonseed, soya bean, olive,

| Concentrate        |                               |                            | Tailing            |                               |                            | Promoter                                              | Lbs./ton | Frother <sup>1</sup> ,<br>lbs./ton |
|--------------------|-------------------------------|----------------------------|--------------------|-------------------------------|----------------------------|-------------------------------------------------------|----------|------------------------------------|
| Per cent<br>weight | Per cent<br>CaCO <sub>3</sub> | Dist.<br>CaCO <sub>3</sub> | Per cent<br>weight | Per cent<br>CaCO <sub>3</sub> | Dist.<br>CaCO <sub>3</sub> |                                                       |          |                                    |
| 94.58              | 74.15                         | 97.68                      | 5.42               | 30.77                         | 2.32                       | K—coconut oil soap.....                               | 0.76     | 0.128                              |
| 83.14              | 81.04                         | 94.67                      | 16.86              | 22.51                         | 5.33                       | Na—coconut oil soap.....                              | 0.50     | 0.064                              |
| 88.54              | 78.42                         | 97.28                      | 11.46              | 16.94                         | 2.72                       | Na—coconut oil soap.....                              | 0.54     | 0.128                              |
| 82.54              | 79.71                         | 92.74                      | 17.46              | 29.52                         | 7.26                       | NaOH and coconut oil fatty acid added separately..... | 0.54     | 0.128                              |
| 85.78              | 74.55                         | 89.38                      | 14.22              | 53.40                         | 10.62                      | K—coconut oil soap.....                               | 0.38     | 0.128                              |
| 70.79              | 82.77                         | 82.62                      | 29.21              | 42.20                         | 17.33                      | Na—coconut oil soap.....                              | 0.38     | 0.128                              |
| 34.29              | 79.10                         | 39.45                      | 65.71              | 65.70                         | 60.55                      | Na—cottonseed oil soap.....                           | 0.38     | 0.128                              |

<sup>1</sup> The frother used in the tests was a mixture of branched and straight chain aliphatic monohydric alcohols boiling between about 150° C. and about 165° C. obtainable by the catalytic hydrogenation of carbon oxides.

An examination of the results in the above table shows that .54 lb./ton of the sodium soap of coconut oil resulted in a recovery of calcite approximately equivalent to that obtained using .76 lb./ton of the corresponding potassium soap and at the same time produced a much higher grade concentrate. This shows that the sodium soap is a more selective promoter for calcite than is the corresponding potassium soap. Similarly the results produced by the sodium soap are better than the free fatty acids and also that the addition of the sodium soap as such to the flotation pulp is better than adding the fatty acid and caustic soda separately to the pulp.

Additional tests were run in which the carbon was floated off first by means of 0.128 lb. of frother per ton of ore. All of the promoter was then added and the resulting concentrate was skimmed off for two minutes. In the tests using the free acids the NaOH was added separately. The results of these tests are given in the following table.

peanut, corn, and similar oils, which contain less than one fourth fatty acids having less than 18 carbon atoms, are not. We have also been able to show that the sodium soaps of individual fatty acids containing 16 or less carbon atoms are efficient calcite promoters. This could not have been predicted since it is known that non-metallic ore materials, such as for example phosphate rock, cannot be effectively promoted with the low molecular weight fatty acids.

In the processing of cement raw materials it is very important that the reagents employed be relatively inexpensive. We, therefore, prefer to use the sodium soaps produced by saponifying natural mixtures of fatty acid glycerides in which at least one third of the fatty acids present consist of fatty acids containing not more than 16 carbon atoms. Representative members of the preferred sodium soaps are those of coconut oil, palm kernel oil, and palm oil since the proportion of high molecular weight fatty acids, that is to say, those having 18 or more carbon atoms,

| Feed,<br>per cent<br>CaCO <sub>3</sub> | Concentrate        |                               |                                            | Tailing,<br>per cent<br>CaCO <sub>3</sub> | Promoter                 | Lbs./ton |
|----------------------------------------|--------------------|-------------------------------|--------------------------------------------|-------------------------------------------|--------------------------|----------|
|                                        | Per cent<br>weight | Per cent<br>CaCO <sub>3</sub> | Recovery,<br>per cent<br>CaCO <sub>3</sub> |                                           |                          |          |
| 70.88                                  | 80.15              | 75.99                         | 85.92                                      | 33.10                                     | Na—coconut oil soap..... | 0.50     |
| 73.99                                  | 53.62              | 81.22                         | 58.86                                      | 66.03                                     | Fish oil fatty acid..... | 2.00     |
| 74.09                                  | 23.57              | 77.74                         | 24.73                                      | 73.42                                     | Talloel.....             | 2.00     |

constitute not more than two thirds of the fatty acids present.

We claim:

1. The method of concentrating calcite by froth flotation which comprises subjecting an aqueous ore pulp containing calcite and siliceous gangue minerals to froth flotation in the presence of a reagent selected from the group consisting of the sodium soaps of fatty acids containing from 8 to 16 carbon atoms and the sodium soaps of mixtures of fatty acids in which at least one third of said mixture consists of fatty acids containing not more than 16 carbon atoms, said froth flotation being carried out in the absence of calcite activators.

2. The method of concentrating calcite by froth flotation which comprises subjecting an aqueous ore pulp containing calcite and siliceous gangue minerals to froth flotation in the presence of sodium soaps of fatty acids containing from 8 to 16 carbon atoms, said froth flotation being carried out in the absence of calcite activators.

3. The method of concentrating calcite by froth flotation which comprises subjecting an aqueous ore pulp containing calcite and siliceous gangue minerals to froth flotation in the presence of sodium soaps of mixtures of fatty acids in which at least one third of said mixture consists of fatty acids containing not more than 16 carbon atoms, said froth flotation being carried out in the absence of calcite activators.

4. The method of concentrating calcite from argillaceous limestones, marls and chalks which comprises subjecting an aqueous pulp of the ore to froth flotation in the presence of a collector for the calcite, said collector being selected from the group consisting of the sodium soaps of fatty acids containing from 8 to 16 carbon atoms and the sodium soaps of mixtures of fatty acids in which at least one third of said mixture consists of fatty acids containing not more than 16 carbon atoms, said froth flotation being carried out in the absence of calcite activators.

5. The method of concentrating calcite from

argillaceous limestones, marls, and chalks which comprises subjecting an aqueous pulp of the ore to froth flotation in the presence of sodium soaps of fatty acids containing from 8 to 16 carbon atoms, said froth flotation being carried out in the absence of calcite activators.

6. The method of concentrating calcite from argillaceous limestones, marls, and chalks which comprises subjecting an aqueous pulp of the ore to froth flotation in the presence of sodium soaps of mixtures of fatty acids in which at least one third of said mixture consists of fatty acids containing not more than 16 carbon atoms, said froth flotation being carried out in the absence of calcite activators.

7. The method of concentrating calcite from argillaceous limestones, marls, and chalks which comprises subjecting an aqueous pulp of the ore to froth flotation in the presence of the sodium soaps of coconut oil fatty acids, said froth flotation being carried out in the absence of calcite activators.

8. The method of concentrating calcite from argillaceous limestones, marls, and chalks which comprises subjecting an aqueous pulp of the ore to froth flotation in the presence of the sodium soaps of palm oil fatty acids, said froth flotation being carried out in the absence of calcite activators.

9. The method of concentrating calcite from argillaceous limestones, marls, and chalks which comprises subjecting an aqueous pulp of the ore to froth flotation in the presence of the sodium soaps of palm kernel oil fatty acids, said froth flotation being carried out in the absence of calcite activators.

10. A process according to claim 1 in which the reagent is stage fed into the aqueous ore pulp.

11. A process according to claim 1 in which carbonaceous material is removed from the ore pulp prior to the froth flotation concentration of the calcite.

DAVID WALKER JAYNE, JR.  
STEPHEN EDWARD ERICKSON.  
HAROLD MILTON DAY.